

## UNITED STATES PATENT OFFICE

2,052,142

## SILVER ALLOYS

Edward F. Kern, New York, N. Y., assignor to  
 The American Metal Company, Limited, New  
 York, N. Y., a corporation of New York

No Drawing. Application August 20, 1935,  
 Serial No. 36,962

2 Claims. (Cl. 75—173)

This invention relates to the production of tarnish-resisting silver alloys of a fineness equivalent to sterling 925 and standard quality 900 fine, as well as the composition of other silver 5 alloys possessing tarnish-resisting properties.

It is well-known that silver alloys and articles made of silver when exposed to the atmosphere or when in contact with substances containing sulfur assume a darkened color known as tarnish.

10 The object of this invention is to provide silver alloys of fineness of sterling quality and otherwise which possess tarnish resisting properties and also which may be readily made into articles which possess sufficient hardness to withstand the usual wear and tear.

15 The invention comprises the novel compositions and component mixtures comprised in such compositions, specific embodiments of which are described hereinafter by way of example only and in accordance with what I now consider the preferred manner of practicing the invention.

20 This application is a continuation in part of my copending application Ser. No. 739,295, filed August 10, 1934.

25 The invention comprises a homogeneous tarnish-resisting silver-tin alloy, with said component metals ranging respectively from 85 to 93% and from 3 to 14%, totaling not more than 99% and not less than 94% of the alloy 30 and silicon in an amount not exceeding 1% and holding in solid solution as the remainder of the alloy one or more workability control metals, cadmium, zinc, antimony, nickel-chromium alloy, copper, manganese, selected in such amounts as 35 will insure to the resulting alloy a Brinell hardness of not less than 36. It also includes such an alloy containing silver about 85 to 93%, tin about 3 to 14%, and not more than 1% of silicon. The amount of silicon used is preferably 40 such that up to about 0.7% is found in the resulting finished alloy. The proportion of silicon may exceed 0.7% up to 1% if desired. A certain amount of silicon is apt to be lost in melting depending on the technique 45 employed in its addition and it is, therefore, well to add a somewhat larger amount thereof to the mixed melt than expected in the resulting alloy. As stated this additional amount will depend on the technique employed and can be readily determined for a given case by making one or more melts and observing the resulting amount of such 50 metal obtained in the finished melt. The proportions above given produce homogeneous solid alloys. The proportion of copper should not exceed about 3.5%. In preparing the above alloys

it is important that they be substantially homogeneous throughout. The proportions given above produce homogeneous solid alloys. Heterogeneous combinations do not possess the desired properties and I, therefore, have selected the 5 homogeneous compositions given.

As regards the specific effect of the metals present in silver alloys the properties were determined by testing a series of the alloys. Tin forms homogeneous solid solution alloys with silver up to 15% tin and 85% silver. Tin increases the hardness and lowers the melting point of the resulting alloy. Other elements as specified above impart tarnish-resisting properties to the alloy and also increase the hardness of the resulting 15 alloy.

The results of the tests demonstrated that the silver-tin alloys are more tarnish-resisting than the silver-zinc and silver-antimony alloys. The inclusion of small amounts of silicon, cadmium, 20 zinc, antimony, manganese, copper, or nickel-chromium alloy in silver-tin alloys increases their tarnish-resisting properties. Silicon added to alloys of silver-tin with small amounts of cadmium, zinc, antimony and copper further increase the 25 tarnish-resisting properties and hardness.

Cadmium, zinc, antimony, copper, manganese and nickel-chromium alloy added to silver-tin alloys control the workability of the resulting 30 alloys.

The compositions made up embodying the metals indicated above were tested to determine their tarnish-resisting properties as follows:—A small cast block of the composition to be tested was rolled into sheets, highly polished and covered by a water solution of ammonium sulfide containing an excess of free sulfur. This solution of ammonium sulfide and sulfur was selected from a number of tarnish-producing materials, as the most active of the various agents tested. The 35 most satisfactory solution of ammonium sulfide and free sulfur consisted of an N/10 ammonium sulfide plus N/100 excess free sulfur. The expressions N/10 and N/100 are intended to designate respectively 10th normal and 100th normal 40 solutions. In accordance with the standard practice a normal solution is one containing an equivalent weight in grams of the substance dissolved in one liter of water or other solvent. The specimen was kept in contact with this solution for 50 five minutes, then washed and dried. The tarnish was then observed on the specimen. When identical specimens were exposed to the atmosphere for several months, the tarnish-resisting effects observed corresponded to those obtained 55

in the much shorter interval required by the above test.

As noted above the alloys vary in their hardness according to their composition and I have tested this hardness in accordance with the well known Brinell test, the test being applied to the alloys as cast. The Brinell test on sterling silver as such, containing 92.5% silver and 7.5% copper shows a hardness of 67, as cast. I find that alloys having tarnish-resisting properties can be produced with the hardnesses indicated for sterling silver or with hardnesses which are less or greater than sterling silver.

I give below a series of alloys prepared in accordance with my invention, together with the results of the above tarnish test and the Brinell hardness test made on the alloy as cast.

| Example No. | Composition of mixtures—Melted—Parts by weight        | Brinell hardness |
|-------------|-------------------------------------------------------|------------------|
| 20          |                                                       |                  |
| 1           | 90 silver, 9 tin, 1 silicon.....                      | 58               |
| 2           | 90 silver, 9.3 tin, 0.7 silicon.....                  | 68               |
| 3           | 89.5 silver, 8.75 tin, 1.65 cadmium, 0.1 silicon..... | 45               |
| 4           | 88.6 silver, 8.5 tin, 2.5 cadmium, 0.4 silicon.....   | 52               |
| 5           | 90 silver, 6.8 tin, 2.5 cadmium, 0.7 silicon.....     | 54               |
| 6           | 90 silver, 8.3 tin, 1 cadmium, 0.7 silicon.....       | 70               |
| 7           | 90 silver, 8.2 tin, 1.5 cadmium, 0.3 silicon.....     | 50               |
| 8           | 90 silver, 8.1 tin, 1.5 cadmium, 0.4 silicon.....     | 50               |
| 9           | 90 silver, 7.8 tin, 1.5 cadmium, 0.7 silicon.....     | 60               |
| 10          | 90 silver, 7.5 tin, 1.5 cadmium, 1 silicon.....       | 69               |
| 11          | 90.3 silver, 7.8 tin, 1.5 cadmium, 0.4 silicon.....   | 48               |
| 12          | 87.5 silver, 7 tin, 5 cadmium, 0.5 silicon.....       | 57               |
| 13          | 90 silver, 6.8 tin, 2.9 cadmium, 0.3 silicon.....     | 40               |
| 14          | 90 silver, 6.6 tin, 2.7 cadmium, 0.7 silicon.....     | 57               |
| 15          | 92.5 silver, 6 tin, 1.2 cadmium, 0.3 silicon.....     | 27               |
| 16          | 90 silver, 5.5 tin, 3.8 cadmium, 0.7 silicon.....     | 55               |
| 17          | 90 silver, 8.3 tin, 1 zinc, 0.7 silicon.....          | 50               |
| 18          | 90 silver, 7.8 tin, 1.5 zinc, 0.7 silicon.....        | 50               |
| 19          | 90 silver, 7.5 tin, 1.75 zinc, 0.75 silicon.....      | 62               |
| 20          | 90 silver, 7.3 tin, 2 zinc, 0.7 silicon.....          | 65               |
| 21          | 90 silver, 7.5 tin, 2 zinc, 0.5 silicon.....          | 54               |
| 22          | 90 silver, 6.3 tin, 3 zinc, 0.7 silicon.....          | 65               |
| 23          | 90 silver, 5.5 tin, 3.8 zinc, 0.7 silicon.....        | 63               |
| 24          | 90 silver, 7.1 tin, 2.5 copper, 0.4 silicon.....      | 56               |
| 25          | 90 silver, 7 tin, 2.5 copper, 0.5 silicon.....        | 55               |
| 26          | 90 silver, 6.5 tin, 2.5 copper, 1 silicon.....        | 58               |
| 27          | 90 silver, 6.5 tin, 2.75 copper, 0.75 silicon.....    | 67               |
| 40          | 90 silver, 6.25 tin, 3.25 copper, 0.5 silicon.....    | 60               |
| 28          | 90 silver, 8.7 tin, 1 antimony, 0.3 silicon.....      | 64               |
| 29          | 90 silver, 8.8 tin, 1 antimony, 0.2 silicon.....      | 50               |
| 30          | 90 silver, 8.2 tin, 1.5 antimony, 0.3 silicon.....    | 61               |
| 31          | 90 silver, 8 tin, 1.3 antimony, 0.7 silicon.....      | 69               |
| 32          |                                                       |                  |

45 The alloys prepared as indicated in the above examples all showed by appropriate tests that they were substantially homogeneous alloys, being substantially free from heterogeneous structure. Each of the alloys of the above examples, 50 when subjected to the ammonium sulfide and sulfur tests indicated above, had a tarnish-resisting property capable of resisting such treatment substantially without appearance of tarnish. Sterling silver and standard silver and various other 55 silver alloys when subjected to this test showed

appreciable tarnish. The silver employed in the above melts was a fine commercial electrolytic silver as crystals of a high grade of purity and the other metals were also commercial products of high purity.

5 The following process is carried out in forming the alloys of the metal or metals with silver and tin:—

10 The alloys are prepared by melting the weighed amounts of electrolytic silver and the other constituents under a flux of for example borax, or glass, and charcoal. The molten mixtures are thoroughly mixed, then cast in the usual manner. When silicon is made a constituent of the alloy, it may be added either as previously prepared alloys, or the silver alloy of silicon may first be prepared, and then the other constituents added. It is found that silicon can be easily incorporated with silver by placing a layer of the electrolytic silver crystals in the crucible, placing 15 the silicon on the layer of silver and covering with the remaining electrolytic silver. In the case of silicon, the combination results when the silver is entirely melted.

15 While I have described my improvements in great detail and with respect to certain preferred embodiments thereof, I do not desire to be limited to such details or embodiments since many changes and modifications may be made and the invention embodied in widely different forms 20 without departing from the spirit and scope thereof in its broader aspects. Hence I desire to cover all equivalents and all modifications and forms coming within the language or scope of any one or more of the appended claims.

25 What I claim as new and desire to secure by Letters Patent, is:—

1. A homogeneous tarnish-resisting silver-tin alloy with said component metals ranging respectively from 85 to 93% and from 3 to 14%, 40 totaling not more than 99% nor less than 94% of the alloy, with silicon not exceeding about 1.0% and holding in solid solution as the remainder of the alloy one or more workability-control metals, cadmium, zinc, antimony, nickel-chromium alloy, 45 copper, manganese, selected in such amounts as will insure to the resulting alloy of Brinell hardness of not less than 36.

2. A tarnish-resisting silver alloy containing silver about 85-93% by weight, an appreciable 50 amount but less than about 1.0% of silicon, and 1 to 5% of a metal selected from the group cadmium, zinc, antimony, nickel-chromium alloy, manganese, and tin constituting the remainder.

EDWARD F. KERN. 55